

## 1

2,831,749

**METHOD OF STERILIZING PLASTER OF PARIS  
SURGICAL DRESSINGS**

Armand M. Marinaro, Wildwood Crest, and Leo Brickman, Metuchen, N. J., Jane E. Smith Holden, Fort Bragg, N. C., and Mary Anne D. Vickery, New Brunswick, N. J., assignors to Johnson & Johnson, a corporation of New Jersey

No Drawing. Application November 15, 1954  
Serial No. 468,994

8 Claims. (Cl. 21—57)

This invention relates to sterilization of plaster of Paris bandages.

Plaster of Paris is the hemihydrate of calcium sulphate and is commercially prepared by heating gypsum ( $\text{Ca}_2\text{SO}_4 \cdot 2\text{H}_2\text{O}$ ) to remove a portion of the water of crystallization to form the hemihydrate plaster of Paris ( $\text{Ca}_2\text{SO}_4 \cdot \frac{1}{2}\text{H}_2\text{O}$ ). When the plaster of Paris is mixed with water, the hemihydrate rehydrates to gypsum and forms a hard solid mass or cast. This phenomenon is known as setting plaster of Paris, and time taken to form the cast is known as the setting time of plaster.

Extensive use of these properties of plaster of Paris is made in orthopedic bandages. The bandage comprises particles of plaster of Paris adhered to crinoline or other type of backing material. In use, the bandage is dipped in water for a short time by the physician or surgeon, squeezed to express excess water and then wrapped around the portion of the body of the patient and allowed to set up as a cast. Plaster of Paris orthopedic bandages should have a fast setting time for this enables the doctor to shorten the time that the patient must be held in traction while the plaster hardens. Furthermore, a cast thus formed should have good high initial cast strength so that when the patient is removed from the operating or cast room, the cast will not break down and the member will remain immobilized.

Requirements of the medical profession with respect to quality of surgical dressings have become more stringent and exacting the past few years. Accordingly, efforts have been made to sterilize plaster of Paris bandages just as most other surgical dressings are sterilized before use. In conventional methods of sterilization, live wet steam under pressure, or several treatments of boiling water, are usually employed. In these cases it becomes extremely difficult, if not impossible, to prevent contact or condensation of moisture on the plaster, as a result of which the useful qualities of the bandage, by reason of the properties of plaster of Paris, enumerated above, are impaired or destroyed. For example, as a plaster of Paris bandage is autoclaved in the conventional manner with 15 to 20 lbs. steam gauge pressure for 30 minutes, the bandage, upon removal from the autoclave, is found to be greatly retarded in setting time beyond the period which would be found to be useful by the orthopedic surgeon. A bandage so treated, which may have an original setting time of 5 to 8 minutes, after treatment in the autoclave does not set within an hour, if at all.

Objects of the present invention include provision of a process for sterilizing plaster of Paris bandages without impairing the qualities of setting time and cast strength upon which the usefulness of plaster of Paris in orthopedic work depends.

A further object of the invention is to sterilize the plaster of Paris bandage in such a manner that the bandage, properly handled, will retain its sterility indefinitely.

According to the invention, plaster of Paris bandages are sterilized by sealing them in a container impermeable

## 2

to water vapor and microorganisms, and heating them in the container in the presence of an amount of water controlled below a certain maximum level, at temperatures set forth below and time to bring about sterilization.

5 A particular embodiment of the invention is directed to additional use of a certain chemical sterilizing agent, in which case water vapor content and temperature may be advantageously maintained at certain lower levels.

The presence of water in the sterilization container is 10 necessary to kill all the microorganisms. According to the invention, sterility is produced without resultant degradation of the plaster of Paris due to water by controlling the amount of water present in the system at a value not greater than 1.1 parts by weight per 100 parts

15 of the weight of the plaster of Paris. When, in addition to the water, certain amounts of chemical sterilizing agent are added according to an embodiment of the invention hereinafter described, water content may advantageously be maintained at a level not greater than 0.55 part per 100 parts by weight of plaster of Paris. The minimum amount of water to produce sterility will vary from 0.13 part per 100 parts by weight of plaster of Paris when chemical sterilizing agent is utilized, to 0.5 part when there is no chemical sterilizing agent present. Accordingly, generally speaking, the minimum amount of water present will be at least 0.13 part, and sufficient to sterilize.

The necessary amount of water may be introduced by means of a hydrated salt which may liberate water of crystallization at the elevated temperatures used for sterilization. Examples of salts of this nature are gypsum, Epsom salts, washing soda, etc. The amounts of such a salt utilized are those equivalent to the amounts of water set forth above. The water or water-yielding salt is added to the sterilizing container in such a manner as not to come into direct contact with the plaster of Paris.

Another variable in the process is temperature, which is sufficiently high so that under the conditions maintained, sterility will result. Without the assistance of a chemical sterilizing agent, temperatures at or above about 40 240° F. may be found necessary to sterilize within a reasonable time. With a chemical sterilizing agent, temperatures above about 212° F. may be found effective. Hence, generally speaking, satisfactory temperatures are those at or above 212° F. at which the system may be sterilized under the conditions maintained therein. Temperatures as high as 290° F. may be used, but above this level some discoloration and deterioration of the bandage, and, in particular, the backing material for the bandage, may take place. The temperature is maintained at a level, and the sterilizing conditions prevail, for sufficient time to kill all microorganisms, a balance being chosen between shorter sterilization times in the range of one to two hours at the higher temperatures, and longer sterilization times but without deterioration of the bandage at the lower temperature levels.

As indicated above, a particular embodiment of the invention is directed to use of a chemical sterilizing agent, notably formaldehyde. Formaldehyde may be used as such, e. g. as an aqueous solution, formalin, or as a chemical which, when heated, produces formaldehyde, e. g. para-formaldehyde. The amount of formaldehyde-producing material sufficient to yield at least about 0.13 part of formaldehyde ( $\text{HCHO}$ ) per 100 parts by weight of plaster of Paris, the minimum amounts of water and the minimum temperature levels being those outlined above, i. e. at least about 212° F. and 0.13 part of water per 100 parts by weight of plaster. A scavenger may be added to the sterilizing container to destroy residual formaldehyde. Such a material is, for example, urethane.

70 The following examples, demonstrating the manner in which the invention method is carried out, are presented as illustrating rather than limiting the invention.

**3**  
**Example I**

4" by 5 yd. commercially available plaster of Paris orthopedic bandage rolls were in all cases utilized. A strip of gauze inoculated with highly resistant spore-bearing organisms was added to each bandage roll. All materials were dried at 45° C. for 16 hours beforehand in order to remove all traces of free moisture. The bandage was placed in a steel container to which there had already been added a predetermined amount of water or water-yielding salt. A grid or stand had been placed on the bottom of the container to prevent the bandage from coming into contact with the water or water-yielding salt and absorbing or reacting therewith. The container was sealed and then heated in a hot air oven at a predetermined time and at a predetermined oven temperature. After allowing the bandage to cool for 24 hours, each of the bandages was tested for setting time and cast strength as described in Federal Specification GG-B-107, paragraphs 4.3.5. and 4.3.6. Sterility testing was carried out according to USP XIV. The results are summarized in the following table:

| Test | Water Added (Parts per 100 of Bandage) <sup>1</sup> | Temp., ° F. | Sterilizing Time, hrs.        | Setting Time, min.             | 1 hour Cast Strength, lbs. | Sterility    |
|------|-----------------------------------------------------|-------------|-------------------------------|--------------------------------|----------------------------|--------------|
| 1.   | 0                                                   | 265         | 2                             | 6 <sup>1</sup> / <sub>4</sub>  | 460                        | Not sterile. |
| 2.   | 0.22                                                | 265         | 2                             | 6                              | 420                        | Do.          |
| 3.   | 0.33                                                | 265         | 2                             | 6 <sup>1</sup> / <sub>2</sub>  | 440                        | Do.          |
| 4.   | 0.45                                                | 265         | 2                             | 6                              | 410                        | Sterile.     |
| 5.   | 0.45                                                | 265         | 2                             | -----                          | -----                      | Not sterile. |
| 6.   | 0.45                                                | 265         | 2 <sup>1</sup> / <sub>2</sub> | 14                             | 402                        | Sterile.     |
| 7.   | 0.45                                                | 290         | 2                             | 13                             | 384                        | Do.          |
| 8.   | 0.55                                                | 265         | 2                             | 11                             | 417                        | Do.          |
| 9.   | 0.89                                                | 265         | 2                             | 20                             | 342                        | Do.          |
| 10.  | 0 Water-1-3.85 Gypsum.                              | 265         | 2                             | 11 <sup>1</sup> / <sub>2</sub> | 337                        | Do.          |
| 11.  | Untreated Controls                                  | -----       | -----                         | 7 <sup>1</sup> / <sub>4</sub>  | 462                        | Not sterile. |

<sup>1</sup> Bandages were 90% plaster of Paris, 10% fabric, by weight.

**Example II**

The procedure outlined in Example I was repeated, except that a formaldehyde-yielding material and, in some cases, a formaldehyde scavenger (urethane), was also incorporated in the sterilizing container. After the heat treatment the bandages were allowed to cool for 24 hours, and tested for sterility, setting time and cast strength according to the procedures presented in Example I. Results are presented in the following table:

| Test | Additives (Parts per 100 of Bandage) <sup>1</sup> | Sterilizing Time, hrs. | Temperature, ° F. | Setting Time, min.             | 1 hour Cast Strength, lbs. | Sterility    |
|------|---------------------------------------------------|------------------------|-------------------|--------------------------------|----------------------------|--------------|
| 1.   | 0.13 paraformaldehyde                             | 2                      | 212               | 4 <sup>1</sup> / <sub>2</sub>  | 405                        | Not sterile. |
| 2.   | 0.22 paraformaldehyde                             | 2                      | 212               | 5                              | 385                        | Do.          |
| 3.   | 0.67 urethane                                     | 3                      | 212               | 4                              | 392                        | Do.          |
| 4.   | 0.67 urethane, 0.22 water                         | 3                      | 212               | 6 <sup>1</sup> / <sub>4</sub>  | 360                        | Do.          |
| 5.   | 0.67 urethane, 0.22 paraformaldehyde              | 3                      | 212               | 5 <sup>1</sup> / <sub>2</sub>  | 350                        | Do.          |
| 6.   | 0.13 paraformaldehyde, 0.22 water                 | 2                      | 212               | 6 <sup>1</sup> / <sub>2</sub>  | 374                        | Do.          |
| 7.   | 0.22 paraformaldehyde, 0.22 water                 | 2                      | 212               | 5 <sup>1</sup> / <sub>2</sub>  | 381                        | Sterile.     |
| 8.   | 0.045 water, 0.22 paraformaldehyde, 0.67 urethane | 3                      | 212               | 3 <sup>1</sup> / <sub>2</sub>  | 335                        | Not sterile. |
| 9.   | 0.13 water, 0.22 paraformaldehyde, 0.67 urethane  | 3                      | 212               | 6 <sup>1</sup> / <sub>4</sub>  | 365                        | Sterile.     |
| 10.  | 0.22 water, 0.22 paraformaldehyde, 0.67 urethane  | 3                      | 212               | 5 <sup>1</sup> / <sub>2</sub>  | 370                        | Do.          |
| 11.  | 0.22 paraformaldehyde, 0.67 urethane, 1.55 gypsum | 3                      | 212               | 6 <sup>1</sup> / <sub>4</sub>  | 352                        | Do.          |
| 12.  | 0.5 water, 0.22 paraformaldehyde, 0.67 urethane   | 3                      | 212               | 10 <sup>1</sup> / <sub>2</sub> | 397                        | Do.          |
| 13.  | 1.0 water, 0.22 paraformaldehyde, 0.67 urethane   | 3                      | 212               | 12 <sup>1</sup> / <sub>2</sub> | 397                        | Do.          |
| 14.  | 2.0 water, 0.22 paraformaldehyde, 0.67 urethane   | 3                      | 212               | 22 <sup>1</sup> / <sub>2</sub> | 360                        | Do.          |

<sup>1</sup> Bandages were 90% plaster of Paris, 10% fabric, by weight.

The foregoing examples show that plaster of Paris bandages may be effectively sterilized consistent with little or no physical or chemical degradation by treatment with an amount of water vapor below a certain

**4**

maximum level, or a chemical sterilizing agent plus certain smaller amounts of water, while maintaining sterilizing temperatures for time sufficient to produce the desired effect.

5 The invention has been described in connection with one embodiment only, but many modifications and equivalents thereof are included within its scope.

The claims are:

1. The method of sterilizing plaster of Paris which comprises treating said plaster of Paris in an enclosed space with water vapor in an amount in the range of about 0.13 to 1.1 parts by weight per 100 parts of plaster of Paris, a formaldehyde providing material in an amount to provide under the treating conditions an amount of formaldehyde in the range of about 0 to about 0.13 part per 100 parts of plaster of Paris, at a temperature in the range of about 212 to 290° F., for a time in the range of about 1 to 3 hours, whereby a sterilized plaster of Paris is obtained having a setting time not over about 22 minutes.

2. The method of claim 1 applied to a plaster of Paris bandage enclosed in a container which is nonporous to micro-organisms.

40 3. The method of claim 2 wherein the amount of formaldehyde is about 0.13 part and the heating is under elevated pressure.

4. The method of claim 3 wherein the container is nonporous to water vapor.

5. The method of claim 4 wherein water is introduced as liquid, and the bandage is supported in the container to avoid direct contact between the liquid water and the plaster of Paris.

6. The method of claim 5 wherein the amount of water is up to about 0.55 part.

7. The method of claim 6 wherein the temperature is at least 240° F. and urethane is included in an amount of

about 0.67 part per 100 parts of plaster of Paris.  
 8. The method of claim 2 wherein the amount of water is at least about 0.5 part and the temperature is at least about 240° F.

## References Cited in the file of this patent

5

UNITED STATES PATENTS  
 830,831 Gronwald Sept. 11, 1906  
 855,942 Duret June 4, 1907

10

1,111,055  
 1,837,264  
 2,009,597  
 2,344,536  
 2,376,611  
 2,472,011  
 2,477,964

510,273

Carveth Sept. 22, 1914  
 Hackley Dec. 22, 1931  
 Weber July 30, 1935  
 Coey et al. Mar. 21, 1944  
 Miner May 22, 1945  
 Graham May 31, 1949  
 Corblin Aug. 2, 1949

## FOREIGN PATENTS

Great Britain July 31, 1939